

## UNITED STATES PATENT OFFICE

CORNELIUS H. KELLER, OF SAN FRANCISCO, CALIFORNIA, ASSIGNOR TO MINERALS SEPARATION NORTH AMERICAN CORPORATION, OF NEW YORK, N. Y., A CORPORATION OF MARYLAND

## FROTH-FLOTATION CONCENTRATION OF ORES

No Drawing.

Application filed January 11, 1928. Serial No. 80,686.

This invention relates to froth-flootation concentration of ores and is herein mainly illustrated as applied to the concentration of ores in which iron occurs in considerable proportion but is essentially a gangue ingredient. In concentrating such ores, especially in concentrating iron-bearing lead-zinc ores and certain copper ores, attempts have been made, by using very small quantities of flotation agents, to inhibit flotation of the iron while at the same time effecting a satisfactory flotation of the more valuable mineral. Such a method of conducting the concentration operation usually requires delicate adjustments and may involve considerable loss of valuable mineral which is dropped in dropping the iron.

According to the present invention a sulphur-containing organic compound is used which is a sulphhydric derivative of a hydrocarbon and which in examples given below shows a marked effect in cooperating with many mineral-frothing agents in facilitating the flotation of the more valuable mineral in a richer concentrate and also in minimizing the flotation of the iron. The invention is herein disclosed in some detail as carried out with ethyl sodium mercaptide, which is a fairly stable crystalline compound, and with para-thio-cresol, with thio-beta-naphthol, with thio-phenol, and with benzyl mercaptan. Another sulphhydric derivative of a hydrocarbon, to wit, ethyl mercaptan itself, has also been found to be an effective reagent for the same purposes.

Other features and advantages will herein-after appear.

Various methods may be found suitable for the commercial preparation of mercaptides, but for the work described herein sodium ethyl mercaptide was prepared by adding metallic sodium to ethyl mercaptan. Mercaptans may be regarded as substituted alcohols, containing sulphur instead of oxygen, thus ethyl mercaptan is  $C_2H_5SH$ . A mercaptide may be regarded as a mercaptan in which the sulphhydric hydrogen is replaced by a metal as in sodium ethyl mercaptide

The following are examples wherein ethyl mercaptide was used:

*Example 1.*—Utah copper ore already ground was further ground for five minutes in a laboratory ball mill with six pounds of lime, measured as calcium oxide, per ton of ore, and was then made into a pulp with the requisite amount of water and agitated for eight minutes in a minerals separation spitzkasten subaeration testing machine with 0.24 pounds of sodium ethyl mercaptide per ton of ore and with one-tenth of a pound of hardwood creosote per ton of ore. The concentrate was separated in the form of a froth and was reagitated with the further addition of three-tenths of a pound of hardwood creosote per ton of ore. The results are shown in the following table:

|            | Assays |       |      | Recoveries |       | 70 |
|------------|--------|-------|------|------------|-------|----|
|            | Wt. %  | Cu %  | Fe % | Cu %       | Fe %  |    |
| Heads..... | 100.0  | 1.01  | 2.64 | 100.0      | 100.0 |    |
| Conc.....  | 2.0    | 36.56 | 23.3 | 72.4       | 19.5  |    |
| Midd.....  | 1.0    | 6.60  | 6.8  | 82.9       | 4.1   |    |
| Tail.....  | 96.4   | .18   | 2.1  | 17.1       | 76.4  | 75 |

*Example 2.*—A four-charge cycle test on another sample of Utah ore showed that there was no tendency to build up either iron or copper in the middlings. The same reagents were used in slightly different quantities, to wit, sodium mercaptide 0.22 pounds per ton, hardwood creosote 0.15 pounds per ton, lime, as CaO, six pounds per ton. This yielded a rougher concentrate which was retreated with a further addition of one-tenth of a pound of creosote per ton of original ore, and produced a finished concentrate and a middling. A second charge was then made up in all respects the same as that for the first treatment and to it was added the middling obtained from the retreatment last described. This yielded a rougher concentrate which was retreated as before to yield a finished concentrate and a middling. A third charge and thereafter a fourth charge were each treated as above described. The concentrates of the four charges were united and assayed as a single product.

The results are shown in the following table:

| 5  | Product     | Assays |       |      | Recoveries |       |
|----|-------------|--------|-------|------|------------|-------|
|    |             | Wt. %  | Cu %  | Fe % | Cu %       | Fe %  |
|    | Heads.....  | 100.0  | 0.60  | 2.26 | 100.0      | 100.0 |
|    | Conc.....   | 2.1    | 21.36 | 25.0 | 75.0       | 23.0  |
|    | Midd.....   | 0.8    | 2.28  | 5.4  | 3.3        | 1.8   |
| 10 | Tail 1..... | 23.4   | 0.12  | 1.6  | 5.0        | 16.4  |
|    | Tail 2..... | 24.2   | 0.12  | 1.3  | 5.0        | 13.7  |
|    | Tail 3..... | 24.6   | 0.12  | 1.9  | 5.0        | 20.8  |
|    | Tail 4..... | 24.9   | 0.14  | 2.2  | 6.7        | 24.3  |

*Example 3.*—A test similar to the first example was carried out with a much smaller amount of sodium ethyl mercaptide. In this test the agitation with lime in the ball mill was the same, the first agitation in the flotation machine was with 0.04 pounds of sodium ethyl mercaptide and 0.2 pounds of hardwood creosote, all per ton of ore, for eight minutes. The concentrate obtained by this treatment was reagitated for three minutes with a further addition of 0.2 pounds of hardwood creosote per ton of original ore. The results are shown in the following table, showing a lower recovery but which was offset by a higher grade of concentrate and an increased rejection of the iron.

| 30 |            | Assays |       |       | Recoveries |       |
|----|------------|--------|-------|-------|------------|-------|
|    |            | Wt. %  | Cu %  | Fe %  | Cu %       | Fe %  |
|    | Heads..... | 100.0  | 1.04  | 2.60  | 100.0      | 100.0 |
|    | Conc.....  | 1.4    | 39.84 | 24.3  | 53.8       | 13.1  |
|    | Midd.....  | 2.0    | 9.48  | 21.98 | 7.0        | 5.4   |
|    | Tail.....  | 96.6   | .30   | 2.2   | 28.1       | 81.5  |

Large rejection of the iron of the ore and richness of the concentrate brought about by the use of a mercaptide are illustrated in the following test of Engels copper ore.

*Example 4.*—The ore was ground fifteen minutes in a laboratory ball mill, and then was made into a pulp and agitated for ten minutes with 2.5 pounds of tri-sodium phosphate (enough to make the pulp alkaline), 0.12 pounds of sodium ethyl mercaptide, and 0.2 pounds of hardwood creosote, all per ton of ore. The resulting froth concentrate was reagitated with 0.3 pounds of hardwood creosote per ton of original ore. The results are shown in the following table:

| 55 |            | Assays |       |      | Recoveries |       |
|----|------------|--------|-------|------|------------|-------|
|    |            | Wt. %  | Cu %  | Fe % | Cu %       | Fe %  |
|    | Heads..... | 100.0  |       |      | 100.0      | 100.0 |
|    | Conc.....  | 3.9    | 33.68 | 14.3 | 73.7       | 5.6   |
|    | Midd.....  | 2.8    | 6.7   | 22.4 | 10.2       | 84.3  |
| 60 | Tail.....  | 93.3   | .30   | 9.7  | 15.7       | 91.5  |

The complex and refractory silver-lead-zinc iron-bearing ore of the San Francisco mines of Mexico yielded rich lead and zinc concentrates relatively free from iron when

concentrated with sodium ethyl mercaptide.

*Example 5.*—The ore was ground for fifteen minutes in a ball mill with half a pound of sodium sulphide per ton of ore. It was then made into a pulp and agitated for seven minutes with three pounds of soda ash, 0.04 pounds of sodium mercaptide, 0.3 pounds of Barrett No. 634 oil, and 0.15 pounds of cresylic acid, all per ton of ore, and a lead-bearing froth was separated. The remainder of the ore pulp was then further agitated for ten minutes with the addition of one-half pound of copper sulphate, 0.1 pounds of sodium mercaptide, 0.3 pounds of Barrett No. 634 oil, and 0.2 pounds of steam distilled pine oil, all per ton of ore, and a zinc-bearing froth separated. The above lead concentrate was separated into a finished concentrate and a middling by reagitation for five minutes with 0.2 pounds of cresylic acid per ton of original ore. The above zinc concentrate was separated into a finished concentrate and a middling by reagitation for three minutes without any added reagent. The results are shown in the following table:

| Assays       |       |               |       |       |      |
|--------------|-------|---------------|-------|-------|------|
|              | Wt. % | Ag. oz. p. t. | Pb %  | Zn %  | Fe % |
| Heads.....   | 100.0 | 21.9          | 10.4  | 22.7  | 6.7  |
| Pb Conc..... | 11.0  | 61.3          | 58.4  | 15.6  | 4.3  |
| Pb Midd..... | 8.5   | 50.8          | 22.8  | 22.9  | 8.8  |
| Zn Conc..... | 28.1  | 23.4          | 3.2   | 51.0  | 8.4  |
| Zn Midd..... | 6.0   | 22.8          | 6.0   | 46.2  | 10.4 |
| Tail.....    | 46.4  | 6.2           | 1.6   | 5.4   | 5.4  |
| Recoveries   |       |               |       |       |      |
|              | Ag %  | Pb %          | Zn %  | Fe %  |      |
| Heads.....   | 100.0 | 100.0         | 100.0 | 100.0 | 105  |
| Pb Conc..... | 30.9  | 61.9          | 7.6   | 7.0   |      |
| Pb Midd..... | 19.7  | 18.7          | 12.1  | 11.2  |      |
| Zn Conc..... | 30.0  | 8.7           | 63.2  | 35.2  |      |
| Zn Midd..... | 6.2   | 3.5           | 6.1   | 9.3   |      |
| Tail.....    | 13.2  | 7.2           | 11.0  | 37.3  |      |

It was found that sodium mercaptide a week old gave nearly the same results as the fresh material.

Extraordinarily complete concentrations have been accompanied by a very large rejection of the iron, as in the following test of California rand ore.

*Example 6.*—The ore was ground in a ball mill for twenty minutes with 3.3 pounds trona (a natural alkali) per ton of ore, and then made into a pulp with water and agitated for fifteen minutes with 0.17 pounds of sodium ethyl mercaptide, 0.33 pounds of coal tar creosote, and 0.17 pounds of steam distilled pine oil, all per ton of ore. The froth concentrate thus obtained was reagitated for four minutes with the further addition of 0.04 pounds of steam distilled pine oil per ton of original ore and yielded a finished concentrate and a middling. The results are shown in the following table:

## Assays

|              | Wt. % | Au oz. p. t. | Ag. oz p. t. | Fe % |
|--------------|-------|--------------|--------------|------|
| 5 Heads..... | 100.0 | .29          | 36.6         | 5.5  |
| Conc.....    | 5.0   | 3.64         | 63.1         | 32.3 |
| Midd.....    | 6.0   | .57          | 31.7         | 11.2 |
| Tail.....    | 89.0  | .08          | 3.6          | 3.5  |

## Recoveries

|               | Au %  | Ag %  | Fe %  |
|---------------|-------|-------|-------|
| 10 Heads..... | 100.0 | 100.0 | 100.0 |
| Conc.....     | 63.3  | 75.2  | 29.4  |
| Midd.....     | 11.9  | 91.3  | 12.2  |
| Tail.....     | 24.8  | 8.7   | 58.4  |

15 It has been found that a sulphhydric derivative of a hydrocarbon is a useful flotation agent in acid and neutral pulps as well as in the alkaline pulps of the above examples.

20 *Example 7.*—Ore of the Allenby Copper Company of British Columbia, containing bornite as the principal copper mineral, was reground for twenty minutes in a ball mill, 25 made into a pulp with water, and agitated with 0.11 pounds of sodium ethyl mercaptide and one-tenth of a pound of cresylic acid, both per ton of ore, and yielded a finished concentrate. The results are shown 30 in the following table:

| Product       | Assays |       |      | Recoveries |       |
|---------------|--------|-------|------|------------|-------|
|               | Wt. %  | Cu %  | Fe % | Cu %       | Fe %  |
| 35 Heads..... | 100.0  | 1.88  | 4.36 | 100.0      | 100.0 |
| Conc.....     | 5.3    | 27.92 | 10.8 | 78.7       | 13.1  |
| Tail.....     | 94.7   | 0.42  | 4.0  | 21.3       | 86.9  |

40 *Example 8.*—Classifier overflow of Anaconda copper ore was reground in a ball mill for five minutes, made into a pulp with water, and agitated for eleven minutes with 0.22 pounds of sodium ethyl mercaptide, one-tenth of a pound of steam distilled pine oil 45 and ten pounds of sulphuric acid, all per ton of ore. The results are shown in the following table.

| Product       | Assays |      |      | Recoveries |       |
|---------------|--------|------|------|------------|-------|
|               | Wt. %  | Cu % | Fe % | Cu %       | Fe %  |
| 50 Heads..... | 100.0  | 1.33 | 4.08 | 100.0      | 100.0 |
| Conc.....     | 13.4   | 9.04 | 24.6 | 91.0       | 80.9  |
| Tail.....     | 86.6   | 0.14 | 0.9  | 9.0        | 19.1  |

50 It has also been found that a sulphhydric derivative of a hydrocarbon is a useful flotation agent when used with such a flotation agent as sodium silicate. It is at times advantageous to add the sodium silicate before the other reagents are added, although this may require a larger quantity of sodium silicate. This procedure has been found to 60 be especially useful in concentrating a cop-

per ore in which a substantial proportion of the copper is oxidized.

65 *Example 9.*—Inspiration ore containing a substantial proportion of oxidized copper was reground for twenty minutes in a ball mill and then made into a pulp with water, and 1.5 pounds of sodium silicate were added to the pulp and mixed therewith. Then were added 0.22 pounds of sodium ethyl mercaptide, 0.6 pounds of hardwood creosote and 0.2 pounds of Barrett coal tar creosote, all per ton of ore, and the pulp agitated for twenty minutes to form a rougher froth concentrate. This concentrate was reagitated for five minutes with half a pound of sodium silicate per ton of original ore, to form a finished concentrate and a middling. The results are shown in the following table:

|            | Assays |       |         |      | Recoveries |         |       |
|------------|--------|-------|---------|------|------------|---------|-------|
|            | Wt. %  | Cu %  | Ox Cu % | Fe % | Cu %       | Ox Cu % | Fe %  |
| Heads..... | 100.0  | 0.89  | 0.22    | 1.81 | 100.0      | 100.0   | 100.0 |
| Conc.....  | 1.4    | 37.42 | 0.68    | 20.4 | 58.4       | 4.5     | 16.0  |
| Midd.....  | 4.7    | 3.22  | 0.54    | 6.4  | 16.9       | 9.1     | 16.6  |
| Tail.....  | 93.9   | 0.24  | 0.20    | 1.3  | 24.7       | 86.4    | 67.4  |

70 In the following example phenol mercaptan or thiophenol was used:

75 *Example 10.*—Impact screen undersize of Utah copper ore was reground with 6 pounds of calcium oxide and with 0.4 pounds of thiophenol, both per ton of the material treated, and was then made into a pulp with water and agitated for ten minutes with 0.4 pounds of dark cresylic acid per ton, and a froth concentrate collected. The results are shown in the following table:

| Product    | Assays |       |      |       | Recoveries |       |
|------------|--------|-------|------|-------|------------|-------|
|            | Wt. %  | Cu %  | Fe % | Cu %  | Fe %       |       |
| Heads..... | 100.0  | 1.25  | 1.36 | 100.0 | 100.0      | 100.0 |
| Conc.....  | 4.42   | 25.76 | 13.5 | 90.8  | 43.8       | 90.8  |
| Tail.....  | 95.58  | .12   | 0.8  | 9.2   | 56.2       | 56.2  |

80 In the following example thio-beta-naphthol was used:

85 *Example 11.*—Impact screen undersize of Utah copper ore was reground with 6 pounds of calcium oxide and 0.4 pounds of thio-beta-naphthol, both per ton of material treated, and was then made into a pulp with water and agitated for ten minutes with 0.55 pounds of dark cresylic acid per ton and a froth concentrate collected. The results are shown in the following table:

| Product    | Assays |       |      |       | Recoveries |       |
|------------|--------|-------|------|-------|------------|-------|
|            | Wt. %  | Cu %  | Fe % | Cu %  | Fe %       |       |
| Heads..... | 100.0  | 1.30  | 1.54 | 100.0 | 100.0      | 100.0 |
| Conc.....  | 5.05   | 23.52 | 13.6 | 91.2  | 44.5       | 91.2  |
| Tail.....  | 94.95  | .12   | 0.9  | 8.8   | 55.5       | 55.5  |

In the following example para-thio-cresol was used:

*Example 12.*—Impact screen undersize of Utah copper ore was reground with 6 pounds of calcium oxide and 0.4 pounds of para-thio-cresol, both per ton of material treated, and was then made into a pulp with water and agitated for ten minutes with 0.9 pounds per ton of dark cresylic acid and a froth concentrate collected. The results are shown in the following table:

| Product    | Assays |       |      | Recoveries |       |
|------------|--------|-------|------|------------|-------|
|            | Wt. %  | Cu %  | Fe % | Cu %       | Fe %  |
| Heads----- | 100.0  | 1.26  | 1.51 | 100.0      | 100.0 |
| Conc.----- | 4.51   | 23.76 | 14.4 | 84.8       | 43.0  |
| Tail-----  | 95.49  | .20   | 0.9  | 15.2       | 57.0  |

Nearly as good results were obtained when the thio-phenol or para-thio-cresol or thio-beta-naphthol were added to the pulp instead of to the material while being ground, although the concentrates were not so rich in copper as when the thio agent was added in the grinding mill.

When potassium phenol mercaptide was substituted for potassium phenol mercaptan or thio-phenol the results of the operation were superior to results obtained in a parallel test wherein it was absent. Similarly, when potassium cresol mercaptide was substituted for potassium cresol mercaptan or thio-cresol the results of the operation were superior to results obtained in a parallel test wherein it was absent.

In the following example benzyl mercaptan was used with a copper ore wherein the iron constituent was negligible:

*Example 13.*—Anaconda table tailings, 65-mesh, were made into a pulp with water and pre-agitated for half a minute in a neutral pulp with 0.32 pounds of pine oil and 0.58 pounds of benzyl mercaptan, both per ton of solids, and then further agitated to yield a froth-concentrate which was separated for three minutes. The results are shown in the following table:

|        | Cu % |                |
|--------|------|----------------|
| Heads  | 1.28 |                |
| Concs. | 7.44 | Recovery 90.1% |
| Tails. | 0.15 |                |

Having now particularly described certain embodiments of my invention, I claim:

1. The process of concentrating an ore containing a mineral value and gangue, which consists in agitating a suitable pulp of the ore containing sodium ethyl mercaptide so as to produce a mineral-value-bearing froth, and separating the froth.
2. The process of concentrating an iron-bearing ore containing a mineral value and gangue, which consists in agitating a suitable pulp of the ore with sodium ethyl mer-

captide so as to form a mineral-value-bearing froth containing a large proportion of a value and a diminished proportion of the iron of the ore, and separating the froth.

3. A method of effecting the concentration of minerals by flotation, which comprises mixing with the mineral pulp a thioalcohol and subjecting the resulting mixture to a froth flotation operation.

4. A method of effecting the concentration of minerals by flotation, which comprises subjecting the mineral pulp to a froth flotation operation in the presence of a nitrogen-free thioalcohol.

5. A process of concentrating ores by flotation which comprises adding to the ground ore a flotation reagent, comprising a compound of the general type  $R-S-R'$ , in which  $R$  stands for an alkyl radical and  $R'$  stands for a metal or hydrogen, and subjecting the mixture to a froth flotation operation.

6. A process of concentrating ores by flotation, which comprises subjecting a pulp of an ore of the mineral to be concentrated to froth flotation in the presence of a mercaptan of the general type  $R-S-H$  in which  $R$  stands for a non-nitrogenous organic radical.

7. The process of concentrating an ore containing a mineral value and gangue, which comprises subjecting a pulp of the ore to froth flotation in the presence of a sulphhydric derivative of a hydrocarbon of the general type  $R-S-R'$ , in which  $R$  stands for an oxygen-free organic radical, and  $R'$  stands for a metal or hydrogen.

8. The process of concentrating an ore containing a mineral value and gangue, which comprises subjecting a pulp of the ore to froth flotation in the presence of a sulphhydric derivative of an aliphatic alkyl group of the general type  $R-S-R'$ , in which  $R$  stands for an oxygen-free organic radical and  $R'$  stands for a metal or hydrogen.

9. A process of concentrating ores by flotation which comprises adding to the ground ore a flotation reagent comprising ethyl mercaptan and subjecting the mixture to a froth flotation operation.

10. A process of concentrating ores by flotation, which comprises adding to the ground ore a flotation reagent, comprising a compound of the general type  $R-S-R'$ , in which  $R$  stands for the ethyl group and  $R'$  stands for a metal or hydrogen.

11. The process of concentrating an iron-bearing ore containing a mineral value and gangue, which consists in agitating a suitable pulp of the ore with a sulphhydric derivative of a hydrocarbon of the general type  $R-S-R'$  in which  $R$  stands for an oxygen-free organic radical and  $R'$  stands for a metal or hydrogen, so as to form a froth containing a large proportion of a value and a diminished proportion of the iron of the ore, and separating the froth.

12. A process of concentrating ores by flotation, which comprises subjecting a pulp of an ore of the mineral to be concentrated to froth flotation in the presence of a mercaptide of the general type R—S—M, in which R stands for a non-nitrogenous organic radical, and M stands for a metal.

5  
In testimony whereof, I have affixed my signature to this specification.

10 CORNELIUS H. KELLER.

15

20

25

30

35

40

45

50

55

60